

1

2,958,590

## STABILIZED HYDROCARBON FUEL OIL COMPOSITION

Joel R. Siegel, Irvington, N.J., assignor to Esso Research and Engineering Company, a corporation of Delaware

No Drawing. Filed Oct. 15, 1957, Ser. No. 690,184

5 Claims. (Cl. 44—62)

The present invention is directed to the stabilization of hydrocarbon oils, and particularly of petroleum middle distillates, against discoloration and the formation of sediment during storage. More particularly, the invention concerns the stabilization of hydrocarbon fuel oils during storage by incorporating into those oils addition agents that inhibit degradation of the fuel oils and which at the same time serve to disperse any sediment-producing materials that may have formed in the fuel oil. The addition agents of this invention are of particular value because they do not form ash or residues when the fuel oils are burned.

The hydrocarbon fuel oils with which this invention is particularly concerned broadly comprise petroleum distillates that are commonly employed in various burner systems, as fuels for diesel engines, as jet fuels and as domestic or industrial heating oils. Such fuel oils may be generally characterized as those that consist of a major proportion of hydrocarbons boiling in the range of from about 350° F. to about 900° F. Fuel oils tend to deteriorate on storage, particularly when they contain cracked hydrocarbon stocks, as they now commonly do. It has been found that if 10 percent or more of the fuel oil composition comprises cracked stocks, the formation of sludge or sediment during storage may be markedly increased, leading to the plugging or fouling of oil lines, filters and burner nozzles.

Attempts have been made in the past to overcome the sediment-forming problem by incorporating addition agents in the fuel oils. Many of these additives, however, particularly metal salts such as metal naphthenates, metal sulfonates and metal salts of alkyl phenol sulfides, have been objectionable in that they leave an ash residue on combustion.

It is a primary object of this invention to improve the stability of petroleum hydrocarbon fuel oils against the formation and precipitation of sediment while at the same time minimizing the formation of ash when such fuels are burned. It is an additional object of the invention to improve the color stability of such fuel oils.

It is still a further object of this invention to provide improved addition agents, and improved methods of preparation of the same, for accomplishing the objects stated above.

In accordance with the present invention, the sediment-forming tendencies of petroleum hydrocarbon oils, and particularly of fuel oils, can be markedly reduced by incorporating therein minor proportions, of the order of from about 0.001% to about 0.2%, of a polymeric material containing an amidine group. The polymeric materials of this invention are preferably prepared by copolymerizing a mixture of three types of monomeric materials, namely, a long chain alcohol ester of a conjugated unsaturated dibasic acid, a vinyl ester of a short chain fatty acid and an N-vinyl amide, and then reacting the resulting copolymer with a primary amine, preferably a tertiary alkyl primary amine. Suitable vinyl esters include vinyl acetate and vinyl propionate. The dibasic

2

acid ester may be a maleate, fumarate, itaconate, aconitate, or the like.

The dibasic acid ester component of the copolymer is preferably an ester of fumaric acid or of mixed fumaric and maleic acids and a long chain alcohol of from about 8 to 24 carbon atoms such as octyl (C<sub>8</sub>), lauryl (C<sub>12</sub>), tridecyl (C<sub>13</sub>), arachidyl (C<sub>20</sub>), behenyl (C<sub>22</sub>), or tallow (C<sub>16-18</sub>) alcohols produced by the hydrogenation of tallow acids.

10 The N-vinyl amide component of the copolymer is characterized by the general structures:



and



where, in the first formula, R is selected from the group consisting of hydrogen and alkyl groups of 1 to 18 carbon atoms and R' is an alkyl group of from 1 to 18 carbon atoms, and, in the second formula, n is an integer from 2 to 4. Preferably R and R' are alkyl groups of 1 to 8 carbon atoms. The second formula given above represents compounds of the first formula wherein R and R' have been replaced by a single divalent hydrocarbon radical of from 2 to 5 carbon atoms to give an internal or cyclic amide.

Among the N-vinyl amides that may be employed in practicing this invention are included N-vinyl-N-methyl acetamide, N-vinyl oleamide, N-vinyl pyrrolidone, N-vinyl-N-isopropyl-2-ethyl hexoic amide, N-vinyl piperidone, N-vinyl-β-methyl pyrrolidone, and N-vinyl-ε-valerolactam.

40 Preferably the copolymers are prepared from mixtures of the monomers in the proportion of about 1 to 1.5 moles of vinyl ester, about 0.5 to 0.7 mole of dibasic acid ester and about 0.5 to 0.3 mole of the N-vinyl amide. Preferably the amounts of the latter two components should add up to about 1 mole for the 1 to 1.5 moles of vinyl ester. The polymerization is conducted in a solution of benzene or other solvent, e.g., xylene, toluene, etc. (50 percent by weight) at temperatures of 60° to 212° F. and may be promoted by gamma radiation or by use of a peroxide type catalyst such as benzoyl peroxide, a hydroperoxide or an azo catalyst such as alpha-alpha'-azo-bis-iso-butyronitrile. The polymerization is conducted until a product of 1000 to 100,000 but preferably 2000 to 20,000 Staudinger molecular weight is produced.

55 The copolymer product after boiling off the solvent is then reacted with a tertiary alkyl primary amine. The amines employed in this invention are preferably those having from about 4 to about 20 carbon atoms. Among the amines that may be used are tertiary octyl primary amine, tertiary dodecyl primary amine, and a commercial mixture of tertiary alkyl primary amines of 12 to 15 carbon atoms, marketed under the name Primene 81R.

60 The copolymer product is reacted with the amine by mixing the product with from 1 to 3 moles, preferably 1.25-2.5 moles, of amine per mole of amide group in the copolymer, the mixture being dissolved in some suitable non-aqueous solvent boiling in the range of about 212° F. to about 350° F., e.g. toluene, xylene. The mix is then refluxed at a temperature of 212-350° F., preferably 230-300° F., for a period of 1-10 hours, preferably 2-6 hours, in a nitrogen atmosphere in the presence of a dehydrating agent such as 1-10% (based on the poly-

mer) of fused zinc chloride or aluminum chloride for example. Alternatively, or in conjunction with the dehydrating agent, the refluxing can be conducted in an apparatus provided with a water separator. The product is filtered, the solvent and excess amine are removed by evaporation in a vacuum and the polymer is redissolved in the desired solvent. In the reaction, the amine group reacts with the amide group of the polymer, forming water and an azomethine group  $>C=N-R$ . The water is removed by distillation or by absorption by the dehydrating agent.

The following examples will serve to illustrate this invention.

#### EXAMPLE 1

Vinyl acetate, tallow fumarate and N-vinyl pyrrolidone in the mole ratio of 1.4/.635/.365 were dissolved in sufficient benzene to make a 50 percent solution by weight. 1.0 percent of benzoyl peroxide was added and polymerization was conducted at 110° F. for 20 hours in the presence of gamma radiation at a dose rate of 1 mr./hr. Then 0.7 mole of tertiary octyl amine (which was an excess) was added along with a quantity of xylene equal in weight to the polymer mix. The blend was refluxed for 4.5 hours in a nitrogen atmosphere in the presence of 8.8 percent anhydrous zinc chloride, based on the polymer. This solution was then filtered, the solvent and excess amine were removed under reduced pressure, and the polymer was dissolved in 50 percent of its weight of benzene. It was established by infrared spectroscope that the amidine grouping was present in the polymer.

#### EXAMPLE 2

A commercial fuel oil was selected for stability tests using the oil itself as well as a blend of the oil containing the additive described in the foregoing example. The oil was a blend of 50 percent virgin distillate and 50 percent cracked stock. Typical inspections for this type of oil are as follows:

|                      |       |
|----------------------|-------|
| Gravity, API         | 30-33 |
| Color (Tag Robinson) | 10    |
| Flash, ° F.          | 130   |
| Sulfur (percent)     | 1.0   |
| Aniline point, ° F.  | 136   |
| Dist. I.B.P. (° F.)  | 315   |
| 10%                  | 392   |
| 50%                  | 479   |
| 90%                  | 581   |
| F.B.P.               | 660   |

The base fuel and the additive blend were subjected to a stability test which consisted in storing the fuel oil for a period of 16 hours while maintaining the temperature at 210° F. At the end of the 16 hours the fuel oil was filtered and the amount of sediment that had been formed during the storage period was quantitatively determined.

Table I sets forth the data obtained in these tests:

Table I  
ACCELERATED STORAGE STABILITY TEST

| Additive                      | Insoluble Sediment Formed After 16 Hours @ 210° F. mg./600 g. Oil |
|-------------------------------|-------------------------------------------------------------------|
| None                          | 12.6                                                              |
| 0.01% of Product of Example 1 | 1.7                                                               |

It will be noted from the data in Table I that the

polymer was very effective in reducing the sediment-forming tendency of the fuel oil.

It is not intended that this invention be limited to the specific examples presented by way of illustration. The scope of the invention is limited only by the appended claims.

What is claimed is:

1. A stabilized hydrocarbon fuel oil composition consisting of a major proportion of hydrocarbons boiling in the range of from about 350° F. to about 900° F., and a minor proportion of a reaction product of a tertiary alkyl primary amine with a copolymer of a vinyl ester of a short chain fatty acid, a long chain alcohol ester of a conjugated unsaturated dibasic acid, and an N-vinyl amide selected from the structural formulas consisting of:



and



wherein R is selected from the group consisting of hydrogen and alkyl groups of 1 to 18 carbon atoms and R' is an alkyl group of from 1 to 18 carbon atoms, and wherein n is an integer from 2 to 4, wherein the amount of vinyl ester utilized is in the range from about 1 to 1.5 moles, wherein the amount of dibasic acid present is in the range from about 0.5 to 0.7 mole and wherein the amount of N-vinyl amide is present in a concentration from about 0.5 to 0.3 mole, said reaction product being present in said hydrocarbon oil composition in an amount sufficient to inhibit the formation of sediment in the said oil.

2. The composition as defined by claim 1 wherein the concentration of the reaction product in the hydrocarbon oil composition is within the range of about 0.001% and about 0.2%.

3. The composition as defined by claim 1 wherein the amine has from 4 to about 20 carbon atoms.

4. The composition as defined by claim 1 wherein the reaction product is obtained from the reaction of from 1 to 3 moles of amine per mole of amido group in the copolymer.

5. The composition as defined by claim 1 wherein said reaction product is prepared from tertiary octyl amine and a copolymer of vinyl acetate, tallow fumarate and N-vinyl pyrrolidone.

#### References Cited in the file of this patent

#### UNITED STATES PATENTS

|           |                  |               |
|-----------|------------------|---------------|
| 2,387,501 | Dietrich         | Oct. 23, 1945 |
| 2,469,737 | McNab et al.     | May 10, 1949  |
| 2,553,325 | Loritsch         | May 15, 1951  |
| 2,597,202 | Lawney           | May 20, 1952  |
| 2,626,945 | Carlin           | Jan. 27, 1953 |
| 2,737,452 | Catlin et al.    | Mar. 6, 1956  |
| 2,771,348 | Meguerian        | Nov. 20, 1956 |
| 2,793,943 | Moore            | May 18, 1957  |
| 2,800,401 | Lusebrink et al. | July 23, 1957 |
| 2,800,452 | Bondi et al.     | July 23, 1957 |

#### FOREIGN PATENTS

|         |         |               |
|---------|---------|---------------|
| 523,748 | Belgium | Nov. 14, 1953 |
|---------|---------|---------------|